

Sept. 7, 1943.

H. E. DEPUTY

2,328,788

## METHOD OF BONDING FERROUS AND NON-FERROUS METALS

Filed Nov. 28, 1941

2 Sheets-Sheet 1



## FIG. I.



FIG.2.

80

HORACE E. DEPUTY

HORACE E. DEPUTY  
Swan, Frey & Hardesty.  
ATTORNEYS

Sept. 7, 1943.

H. E. DEPUTY

2,328,788

METHOD OF BONDING FERROUS AND NON-FERROUS METALS

Filed Nov. 28, 1941

2 Sheets-Sheet 2



FIG.4.



FIG.5.

FIG.6.



FIG.7.



BY

HORACE E. DEPUTY

*Swan, Frye & Hardesty.*  
ATTORNEYS

## UNITED STATES PATENT OFFICE

2,328,788

METHOD OF BONDING FERROUS AND  
NONFERROUS METALS

Horace E. Deputy, Brooklyn, Mich.

Application November 28, 1941, Serial No. 420,781

2 Claims. (Cl. 22—204)

This invention relates to methods of bonding ferrous and non-ferrous metals, constituting a further development of the invention disclosed in my Patent No. 2,123,181, granted July 12, 1938.

An important object of the present invention is to provide an improved method whereby such metals may be intimately and permanently bonded one to the other, in a simple, quick and positive manner which lends itself to rapid production methods, and which enables a large number of such bonding operations to be performed in a short space of time, even though relatively large masses of metal are to be united.

While the invention is illustrated as applied to securing together a steel cylinder and an encircling aluminum sleeve or "muff," adapted to be used in the construction of air-cooled engine cylinders, many other applications will be readily understood to exist.

Other objects and advantages will readily occur to those skilled in the art upon references to the following description and accompanying drawings.

In the drawings:

Fig. 1 is a plan view of a mold assembly adapted to be used in carrying out my improved process.

Fig. 2 is a diametrical cross section taken substantially on the line 2—2 of Fig. 1, and looking in the direction of the arrows.

Fig. 3 is a detail section taken substantially on the line 3—3 of Fig. 1.

Fig. 4 is a central vertical section through the mold taken substantially on the line 4—4 of Fig. 1, and with adjacent supports and mechanism shown in elevation with portions broken away.

Fig. 5 is a diagrammatic plan view of the mold, its supporting stand, and a preferred relative positioning of the cooperating reducing oven and hydraulic press utilized in my improved method.

Fig. 6 is a detail sectional view, taken substantially on the line 6—6 of Fig. 1, showing the mounting of one of the mold heating elements, and

Fig. 7 is a front elevation of a reducing oven used in my improved method.

Referring now to the drawings: The method employed insofar as the formation of the bond itself is concerned, is similar to that disclosed in my Letters Patent No. 2,123,181, above referred to, although additional steps are employed and the rapidity of production of the bonded parts is thereby increased.

In the mold construction shown, a central gen-

erally cylindrical cavity 10 is provided, the external walls of which constitute the outer mold walls for the formation of the "muff" or aluminum sleeve. This is to be cast upon the exterior 5 of a steel cylinder liner or the like, as 12. The liner is adapted to stand in concentric position projecting upwardly from the bottom of the mold, and to form the inner wall of the mold cavity into which the aluminum is poured during 10 casting. The liner 12 is positioned by an annular bottom closure member 13 which defines the bottom of the space 10, but is centrally open to permit escape of the cooling fluid, which is supplied, as will presently be described, through 15 pipe 30.

A pouring sprue 14 leads to the bottom of space 10, and terminates at a gate 15 in an adjacent part of the mold assembly. These parts will be seen to be located upon the parting line of the 20 mold sections, and the general arrangement of these mold parts will be seen to be in accordance with conventional foundry practice. The mold sections 8 and 9 are adapted to be secured together by bolts as 17, the threads and cooperating nuts 18 of which are preferably of the quick opening variety, as shown in Figs. 1 and 3. Electrical or other suitable heating elements 20 may also be incorporated in the mold assembly 25 if desired, to facilitate preheating. As herein illustrated, heating elements 20 of the "globar" type are shown in Figs. 1, 2 and 6. These heating elements 20 extend laterally through the mold sections, and carry terminal clamps 21 at their 30 ends, which connect with suitable flexible electrical conductors, as 22. As shown, a plurality of "globars" are mounted in each mold section.

The top wall of the cavity 10 is defined by another annular closure 25, which is adapted to be lifted by and float upon the poured metal, whereby it may serve as a compression member, through the agency of which pressure may be directly applied to the poured metal to compact the same and collapse any voids which may exist 40 therein.

In carrying out my improved process, the ferrous metal, which in this instance is the steel sleeve or cylinder liner 12, is first preheated to a temperature of 500 to 850° F., in a reducing 50 oven, as 40, after having been previously dipped in a galvanizing bath of molten zinc, preferably of the variety sold commercially, as Western Spelter. As pointed out in my Letters Patent above referred to, the impurities present in this 55 particular material seem greatly to assist in se-

curing uniform bonding (such impurities consisting principally of lead, iron and cadmium).

The galvanized sleeve is guarded against oxidation. It may either be kept hot after galvanizing, and placed in the mold while heated to a temperature of from 500 to 850° F., or may be allowed to cool and then be reheated to bring it to the proper temperature at the time of pouring, but in either event the heating of the galvanized sleeve is preferably effected in a reducing oven, as 40.

The mold is also preheated, to a temperature of from 750 to 850° F. at the time of pouring, and the aluminum is poured at a temperature of approximately 1300° F. The aluminum may either be in the pure state or alloyed with other metals, as desired. Preferably, the pouring is done as quickly as possible after the sleeve is removed from the reducing oven and placed in the mold, so that no opportunity for substantial oxidation of the sleeve is afforded.

After the poured aluminum has been allowed to stand from five to ten minutes, to permit it to solidify in the sprue, pressure is applied to the compression ring 25, to compact the metal in the cavity 10 while it is still relatively soft.

About one minute after pouring commences, also, cooling fluid, such as water, brine, or oil, is directed against the interior of the sleeve 12, through the pipe 30, which projects into the interior of the sleeve and is provided with a plurality of relatively fine orifices 33 arranged to project jets against the interior of the sleeve. Such fluid may be as cool as is available, and, if desired, may be collected after passing through the drain 35 and recirculated. Rapid cooling is possible without interfering with the effectiveness of the bond.

For convenient operation of my method, the mold may be positioned on a suitable stand, as 7, with the quick-opening nuts 18 at the front, as shown in Fig. 5, the fluid control valve 31 being arranged conveniently below the stand top. The reducing oven 40 is preferably mounted at one side of the mold upon a stand, as 41, so that a heated sleeve 12 can be removed through the door 42 and immediately placed in the mold to keep oxidation at a minimum. At the other side of the mold, a hydraulic press 50 may be mounted, as upon a swinging bracket 51 secured on a wall 52. The plunger 53 of the hydraulic press carries a member 54 adapted to contact the annular closure member 25 when swung into position, as shown in dotted lines in Figure 5. The clo-

sure member 25 is preferably formed with a shoulder 26 to limit its travel into the mold aperture 10 and so limit the compression exerted on the soft metal being compacted.

- 5 The application of cooling fluid to the internal surface of the sleeve while the molten aluminum is in contact with the external surface thereof can be arranged to prevent a drawing of the temper of the steel sleeve or softening it 10 beyond the desired Brinnell gauge. This is important when the sleeve is to be used as a liner for an airplane or similar engine cylinders, and the aluminum muff is the air cooling sleeve thereon. By preventing the ferrous sleeve from 15 reaching a temperature sufficient to unduly soften it, is only necessary to maintain the cooling fluid at a sufficiently low temperature, and initiate the flow of the cooling fluid when the sleeve is being heated by the molten aluminum 20 close to the softening temperatures.

I am aware that the invention may be embodied in other specific forms without departing from the spirit or essential attributes thereof, and I therefore desire the present embodiment 25 to be considered in all respects as illustrative and not restrictive; reference being had to the appended claims rather than to the foregoing description to indicate the scope of the invention.

30 I claim:

1. The process of bonding onto a sleeve of ferrous metal a non-ferrous metal, comprising at least partly aluminum, which consists in coating at least the outer periphery of the ferrous sleeve with a coating consisting principally of zinc, preheating the coated surface of the sleeve while limiting access of oxygen to the coated surface, pouring the non-ferrous metal in molten condition into engagement with the coated surface of the sleeve, allowing a time interval of approximately one minute after pouring commences, then projecting a spray of cooling liquid into the interior of the sleeve, allowing a further time interval of at least four minutes, and then 40 applying mechanical pressure to the non-ferrous metal to compact the same and urge it into engagement with the coated surface of the sleeve.
- 45 2. The process set forth in claim 1 wherein the coated ferrous sleeve is preheated to a temperature of from 500 to 850 degrees F., and then placed in a mold preheated to a temperature of from 750 to 850 degrees F. to receive the molten non-ferrous metal.

HORACE E. DEPUTY.